

[54] QUENCHING PROCESS FOR MELT EXTRUDED FILAMENTS

3,129,272 4/1968 Ferrier et al. .... 264/176 Z  
3,553,305 1/1971 Au. .... 264/176 Z

[75] Inventor: Donald Edward Shaffer, Chattanooga, Tenn.

## FOREIGN PATENTS OR APPLICATIONS

[73] Assignee: E. I. Du Pont de Nemours and Company, Wilmington, Del.

44-21169 9/1969 Japan .... 264/176 Z

[22] Filed: Apr. 18, 1974

Primary Examiner—Jay H. Woo

[21] Appl. No.: 462,036

## Related U.S. Application Data

[63] Continuation-in-part of Ser. No. 370,678, June 18, 1973, abandoned.

## [57] ABSTRACT

[52] U.S. Cl. .... 264/176 F; 264/237

Oxidative deposits on a spinneret in a melt spinning process can be reduced by introducing a small amount of a noncondensable inert gas, such as nitrogen, below the steam blanketed zone, but above the point at which quenching air is first directed toward the extruded filaments.

[51] Int. Cl.<sup>2</sup> .... D01D 5/08

[58] Field of Search .... 264/176 Z, 237

## [56] References Cited

9 Claims, 3 Drawing Figures

## UNITED STATES PATENTS

3,053,611 9/1962 Griebl .... 264/176 Z





FIG. 2



**FIG. 3**

## QUENCHING PROCESS FOR MELT EXTRUDED FILAMENTS

### CROSS REFERENCE TO RELATED APPLICATION

This application is a continuation-in-part of my co-pending application, Ser. No. 370,678 filed June 18, 1973 and now abandoned.

### BACKGROUND OF THE INVENTION

This invention relates to melt spinning synthetic polymer filaments. More specifically, this invention provides an improvement in melt spinning processes whereby better continuity of operation is obtained.

The problem of polymer oxidation at the spinneret has long created difficulties when melt spinning synthetic polymers. It is known to provide a blanket of inert gas around the spinneret, to decrease the tendency for oxidized polymer to form around the spinneret orifices. Such deposits must be removed, by the technique termed "wiping" (described hereinafter) else they will interrupt the spinning. Steam has been used for the inert gas, to minimize formation of oxidized polymer.

The molten filaments, after extrusion, are normally cooled by a current of cross flow air or by air which is supplied radially of the filament bundle, and which then flows longitudinally, cocurrent with the filaments' motion. Extreme care is required to minimize exposure of the filaments to turbulent quenching air, since while molten, they are very sensitive to erratic air currents, which may produce denier variations and even cause contact between and fusing of filaments. In some cases, a combination of radially directed and cross flow cooling air has been employed.

Efforts to combine the inert gas blanket and the cooling feature led to the use of cooling with 100 percent inert gas, to quench filaments at a controlled rate, or to processes that combined steam blanketing with carefully controlled cooling air.

In spite of continual efforts to decrease polymer oxidation at the spinneret, it was found impractical to completely eliminate oxygen at the spinneret face; even a very low concentration was enough to cause spinneret deposits with polymers spun at high temperatures, or with those polymers which were easily oxidized.

### SUMMARY OF THE INVENTION

It has been found that oxidative deposits on the spinneret in a melt-spinning process can be reduced below levels heretofore attained, by a process for quenching a melt extruded filament issuing from a spinning pack which comprises introducing immediately below the spinning pack in successive first, second and third zones steam, noncondensable inert gas, and air respectively; and passing the melt extruded filament through said zones to quench the filament.

An additional advantage may be obtained when the inert gas is preheated prior to introduction into said second zone.

### BRIEF DESCRIPTION OF THE DRAWINGS

FIG. 1 represents schematically the apparatus elements employed in the process of the invention.

FIG. 2 shows a quench box arrangement which is adapted to processing four threadlines simultaneously.

FIG. 3 shows an enlarged partial scale-up of the cross section as illustrated in FIG. 1 showing the steam blanketer arrangement in more detail.

### DETAILED DESCRIPTION OF PREFERRED EMBODIMENTS

The process of the invention can be best understood by reference to the drawings. FIG. 1 shows schematically a melt spinning apparatus in which filaments 1 are extruded from a spinneret filter pack 2 from a source of molten polymer, not shown. Filter pack 2 is surrounded by a heated spinning block 3. The filaments are extruded into a steam-blanketed first zone indicated by the numeral 4, supplied with steam from conduit 5. The filaments 1 are cooled as they pass through quench box 6, which is supplied with room temperature air passing through a duct 7 from a source, not shown. The cooling air reaches the filaments by passing through perforations of screen tubes 8, 15 which surround the filament bundle. Tube 8 is formed of perforated metal, and a tube 15 is a double tube consisting of one layer of 20 and two layers of 100 mesh screen. Air is supplied at a rate just equal to the rate at which quiescent air would be aspirated by the moving filaments.

The upper portion of quench box 6 has a partition or baffle plate 12 dividing it into two zones, i.e., second and third zones designated 9 and 10, respectively. Plate 12 is connected to the top flange 14 of the quench box 30 by a seal, which may be flexible as shown at 17 of FIG. 2. Noncondensable inert gas is delivered to zone 9, through conduit 11 and air is delivered to zone 10 through duct 7.

FIG. 2 is a perspective drawing of quench box 6, 35 adapted to furnish quenching air and inert gas to four quench tubes simultaneously. Like numbers denote like parts.

FIG. 3 shows in greater detail the steam blanketed spinneret arrangement in cross section. Again, like 40 numbers denote like parts. In FIG. 3, 2' denotes the filter pack and 2'' the spinneret through which filaments 1 are extruded. Steam is injected through steam conduit 5, into annular slot 19, providing a blanket of steam extending downwardly from the face of spinneret 2''. Annular slot 19 is formed in its lower part by steam blanketer insert 13. Flange 14 of quench box 6 is in sealing contact with blanketer 13. Quench box 6 contains quench tubes 8 and 15, positioned as shown more clearly in FIG. 1.

The maximum amount of cooling air which can be used in any melt spinning process is restricted by the need to protect the filaments from turbulent air currents which may cause filament breaks, fusing and denier variations, as mentioned previously. For the preferred cocurrent quench process disclosed herein, it is desirable that this amount of air correspond to that which is aspirated by the running threadline. This volume of air will vary with number of filaments, size of yarn bundle, and spinning speed. It may be determined empirically, from a study of the relation between yarn defects and air flow rate, or a mathematical model may be devised. The benefits of the instant invention are obtained when a portion of this air is replaced by an inert gas, preferably nitrogen. As will be shown in the examples, optimum improvement in spinning continuity is obtained when from 5 to 20 percent of the quench air is replaced by nitrogen. Surprisingly, replacing larger

amounts of the air with nitrogen appears to provide poorer results, in addition to being more expensive.

It might be hypothesized that a similar improvement could be obtained by increasing the steam flow by an amount corresponding to the volume of nitrogen. This approach is not practical, since the maximum tolerable steam flow is limited by the effect of gas velocity on the freshly extruded filaments; increasing the steam flow next to the spinneret reduces denier uniformity. Introducing additional steam at 11 (FIG. 1) rather than nitrogen when the filaments are cooler, would cause excessive moisture condensation in the quench tube, and, because of condensation, might not reduce oxygen at the spinneret. In addition, cooling with a condensing gas often leads to nonuniformly quenched yarn.

In an attempt to determine the mechanism which produces the benefits of the instant invention, the steam in the blanketer was replaced by an equal volume of (a) heated nitrogen and (b) heated helium, to determine whether a density difference between blanketer and cooling medium was necessary. In both cases, (a) and (b), polymer oxidation at the spinneret was not reduced, indicating that the density difference was not a factor.

In order to achieve the benefits of the invention, baffle 12 should be placed at the optimum position in quench box 6, which position may be empirically determined. However, it is believed that the optimum position for the baffle is controlled by the theoretical considerations described below.

When air is used to cool filaments spun from a steam blanketed spinneret, as in FIG. 1, but without provision for adding inert gas (i.e., partition 12 removed and inlet 11 closed), most of the air introduced radially through screen tubes 8, 15, is immediately carried downward by the moving filaments. In the upper section of the screen tube, however, some of the air eddies upward, mixing with the steam in zone 4, and producing a small oxygen concentration at the spinneret, which causes polymer oxidation around the spinneret orifices. The best location for baffle 12 is believed to be sufficiently far from the spinneret so that none of the air admitted below the baffle will be carried up to the spinneret. This point is believed to lie just below the zone where the upward eddies begin to form.

When using partial inert gas quenching, it will often happen that the lower part (zone 10) of quench box 6 can be dispensed with; the filaments may be cooled by air aspirated through screen tubes 8, 15, or by cross flow air furnished in conventional manner. It is apparent, of course, that when cross flow air is used to cool the filaments, the inert gas should be introduced above the point where the air is first directed toward the filaments.

The process of the instant invention may also be adapted to the various known methods used to delay the cooling of the filaments, for example, by heating the inert gas supplied to zone 9.

Although nitrogen is the preferred inert gas for use in the process of the invention, any nonoxidizing (and, preferably, nontoxic) gas may be used, such as helium, combustion gas and the like.

The principal objective of the invention is to decrease the need to remove oxidized polymer deposits from the face of the spinneret by the technique known as wiping which involves carefully scraping the exposed surface of a spinneret with a brass chisel-like tool. Ob-

viously, this is a costly operation, since it requires hand operation by skilled operators and involves an interruption in production during wiping.

If preventive wiping is not scheduled sufficiently frequently, spinning interruptions will occur; these are of the following types:

- a. a molten filament may spin discontinuously, by dripping from the spinneret orifice;
- b. an occasional thick section of filament is produced;
- c. yarn may break and wrap on the feed roll at the draw zone;
- d. filaments may start to break and wrap on any of the other rolls.

A careful statistical study of the coupled spinning drawing operation is made, and a schedule of preventative wiping is developed to decrease the probability of all interruptions *a-d* to some specified level. The time interval between the preventative wipes determined by this schedule is termed wipe cycle herein; it is taken as a measure of the effectiveness of the gas blanketing system, while all other variables are held constant. Obviously, it is important to increase the wipe cycle as much as possible.

In some tests, the total hours of spinning before an actual interruption by any of (a) to (d) is determined; this period is identified as drip life herein.

The process of the instant invention will be exemplified by a coupled spinning drawing process described

30 by R. H. Knospe in U.S. Pat. No. 3,416,302, which process is used for preparing mixed shrinkage yarns from polymer compositions based on polyamides from bis(4-aminocyclohexyl) methane (abbreviated PACM) and dodecanedioic acid (-12 acid). It is apparent, of course, that the invention may also be advantageously used in the melt spinning of PACM-12 homopolymer alone, or, indeed, for melt spinning any polymer where spinning temperatures are so high (or oxidation resistance so low) that spinning into a steam blanket is used.

#### EXAMPLE I

PACM-12 (70% *tt* isomer) homopolymer and PACM-12-PACM-I copolymer (70% *tt*, also) are prepared essentially as described in Example I of the Knospe patent, U.S. Pat. No. 3,416,302. The polymer and copolymer are then extruded as filaments through separate orifices of a single spinneret, using a quenching chimney as shown in FIG. 1. In this instance, there is only one quench tube assembly 8 within quench box 6, instead of the four tubes shown in FIG. 2. One hundred forty-four filaments (72 of each composition) are extruded into steam blanket zone 4. The filaments are cooled as they pass through nitrogen quench zone 9 and air quench zone 10, after which they are converged into yarn bundles and drawn to a 240 denier yarn, essentially as described in Example I of Knospe, at a yarn windup speed of 2,700 yd./min. (2,550 m./min.). The spinning block temperature is 337°C. The steam blanketer zone 4 is supplied with 0.2 to 0.3 cfm (5.7 to 8.5 l./min.) of steam at 270°C. Nitrogen is supplied at 11 to zone 9 and air at 7 to zone 10.

In two series of tests, various positions of baffle 12 are evaluated, as well as varying amounts of air and nitrogen. The oxygen concentration at the spinneret face is determined, as well as the average drip life under each condition. In all tests, the steam flow is 0.2 to 0.3

cfm (5.7 to 8.5 l./min.) at a temperature of 270°C. The results are listed in Table I.

In Tests 1 and 3, baffle 12 is not in place and air cooling only is employed. In Test 4, air is injected at 11 instead of nitrogen. It should be noted that steam flow is reported as cu. ft./min. measured at 1 atm. and 270°C.

lowing conditions: the spinning block temperature is 332°C.; 1.85 lb/hr (0.87 Kg/hr) steam at 270°C. is supplied to each spinneret blanketer, yarn is spun from each spinneret and after drawing, the yarn is wound up at 3,100 yd./min. (2,830 m./min.). The quenching conditions, air and nitrogen flows, (control employs no inert

TABLE I

| Test No. | Test                | Baffle Position, in. (cm.) <sup>(1)</sup> | N <sub>2</sub> Flow, scfm(l/min) | Air Flow, scfm(l/min) | % Air Repl. <sup>(4)</sup> | O <sub>2</sub> Conc. <sup>(2)</sup> Wt. % | Avg. Drip Life Hrs. |
|----------|---------------------|-------------------------------------------|----------------------------------|-----------------------|----------------------------|-------------------------------------------|---------------------|
| 1        | Control, air        | None                                      | None                             | 63.6(1800)            | None                       | 2.0                                       | 4.5                 |
| 2        | Part N <sub>2</sub> | 3.25(8.25)                                | 27.0(764)                        | 36.6(1004)            | 42                         | 0.8                                       | 9.5                 |
| 3        | Control, air        | None                                      | None                             | 63.6(1800)            | None                       | 3.0                                       | 4.3                 |
| 4        | Air-air             | 1.75(4.44)                                | 7.5 air (212)                    | 56.1(1585)            | None                       | ND <sup>(3)</sup>                         | 4.2                 |
| 5        | Part N <sub>2</sub> | 3.45(8.75)                                | 15(424)                          | 48.6(1375)            | 23                         | 0.7                                       | 12.0                |
| 6        | Part N <sub>2</sub> | 1.75(4.44)                                | 7.5(212)                         | 56.1(1585)            | 12                         | 0.6                                       | 14.9                |

<sup>(1)</sup>Baffle position: distance between baffle 12 and top of quench box 6, inches (and cm.).

<sup>(2)</sup>Oxygen concentration at the spinneret face, wt. %.

<sup>(3)</sup>ND indicates values not determined.

<sup>(4)</sup>% of normal quenching air, replaced by N<sub>2</sub>.

It is observed that oxygen concentration at the spinneret face is significantly reduced, and the average drip life is increased two to three fold. The yarn had good physical properties and denier uniformity.

30

## EXAMPLE II

The test of Example I is repeated on a large scale, using the four-tube quench box of FIG. 2. The spinning block temperature is 337°C.; 0.8 to 1.0 cfm (21.7 to 28.3 l./min.) steam at 270°C. is supplied to each spinneret blanketer. Various filament counts are spun from each spinneret; after drawing, the yarn is wound up at 2,700 yd./min. (2,550 m./min.). In separate runs, polymer with various amounts of kaolinite delusterant (see Iler — U.S. Pat. No. 3,397,171) is employed.

The quenching conditions, air and nitrogen flows, oxygen concentration and wipe cycle are listed in Table II, (test runs 1-8).

It is observed that the addition of nitrogen in the zone above the quench air input reduces oxygen concentration at the spinneret, and increases the wipe cycle. However, as in Example I, it is seen that excessive amounts of nitrogen are frequently less advantageous.

## EXAMPLE III

The procedure of Example II is repeated with the fol-

gas), wipe cycle and drip life are listed in Table II (test runs 9, 10, and 11) which shows that excellent improvement in drip life is obtained when 6 or 11 percent of the quenching air is replaced with nitrogen.

35

## EXAMPLE IV

It may be advantageous to heat the inert gas used to replace a portion of the quenching air, as shown in this example.

40

The procedure of Example III is repeated with the following conditions: the spinning block temperature is 335°C.; 1.75 lbs/hr (0.78 Kg/hr) steam at 280°C. is supplied to each spinneret blanketer; yarn is spun from each spinneret and after drawing, the yarn is wound up at 3,500 yd./min. (3,200 m./min.). The quenching conditions, air and nitrogen flows (control employs no inert gas) wipe cycle and drip life are listed in Table II (test runs 12 and 13). The nitrogen added in Test run 13 is preheated to 200°C., before injection at 11 into second quench zone 9. Increased wipe cycle is observed when 5 percent of the quench air is replaced by heated nitrogen, and in addition, yarn properties are improved.

TABLE II

| Test No. | Test    | Drawn Yarn Count | Kao-linite % | Baffle Posn., in.(cm) | N <sub>2</sub> Flow, scfm(l/m) | Air Flow, scfm(l/min) | % Air Repl. | O <sub>2</sub> Conc. % | Avg. Wipe Cycle, hrs. | Avg. Drip Life hrs. |
|----------|---------|------------------|--------------|-----------------------|--------------------------------|-----------------------|-------------|------------------------|-----------------------|---------------------|
| 1        | Control | 120-72           | 3.3          | None                  | None                           | 50(1780)              | None        | 0.35                   | 15.5                  |                     |
| 2        | Test    | 120-72           | 3.3          | 2.2(5.6)              | 10(280)                        | 50(1780)              | 16          | 0.2                    | 26.5                  |                     |
| 3        | Control | 250-72           | 1.5          | None                  | None                           | 160(4520)             | None        | 0.7                    | 3.4                   |                     |
| 4        | Test    | 250-72           | 1.5          | 1.75(4.44)            | 20(560)                        | 160(4520)             | 11          | 0.14                   | 8.2                   |                     |
| 5        | Test    | 250-72           | 1.5          | 1.75(4.44)            | 30(840)                        | 160(4520)             | 16          | 0.21                   | 6.3                   |                     |
| 6        | Control | 90-30            | 2.0          | None                  | None                           | 110(3110)             | None        | N.D.                   | 7.0                   |                     |
| 7        | Test    | 90-30            | 2.0          | 1.25(3.18)            | 17.0(470)                      | 110(3110)             | 13.4        | 0.22                   | 8.0                   |                     |
| 8        | Test    | 90-30            | 2.0          | 1.25(3.18)            | 17.0(470)                      | 80(2260)              | 17.4        | 0.28                   | 14.0                  |                     |
| 9        | Control | 250-72           | 3.3          | None                  | None                           | 160(4520)             | None        | N.D.                   | 3.3                   | 3.9                 |
| 10       | Test    | 250-72           | 3.3          | 2.5(6.3)              | 10(280)                        | 160(4520)             | 5.9*        | N.D.                   | 8.7                   | 10.8                |
| 11       | Test    | 250-72           | 3.3          | 2.5(6.3)              | 20(560)                        | 160(4520)             | 11.0*       | N.D.                   | 6.6                   | 9.2                 |
| 12       | Control | 180-108          | 3.3          | None                  | None                           | 200(5660)             | None        | N.D.                   | 2.5                   | 4.0                 |
| 13       | Test    | 180-108          | 3.3          | 2.5(6.3)              | 10(283)                        | 190(5370)             | 5.0         | N.D.                   | 9.0                   | 14.0                |

\*nitrogen as a percent of total quench gas

What is claimed is:

1. A process for quenching a melt extruded filament issuing from a spinning pack which comprises introducing immediately below the spinning pack in successive first, second and third zones steam, noncondensable inert gas, and air respectively; and passing the melt extruded filament through said zones to quench the filament.

2. The process as defined in claim 1, wherein said noncondensable inert gas is nitrogen and amounts to from about 5 to about 20 percent of the volume of air being introduced.

3. The process as defined in claim 1, said process being a radial cocurrent quenching process.

4. The process as defined in claim 1, said inert gas being preheated prior to introduction into said second zone.

5. In a process for quenching a melt extruded filament issuing from a spinning pack that includes the

steps of introducing immediately below the spinning pack in successive zones steam and air and passing the filament through the zones to quench the filament, the improvement comprising: replacing a portion of said air being introduced with noncondensable inert gas; and introducing said noncondensable inert gas into a zone between the zones for introducing steam and air.

6. The process as defined in claim 5, about 5 to about 20 percent of said air being replaced by said noncondensable inert gas.

7. The process as defined in claim 6, said noncondensable inert gas being nitrogen.

8. The process as defined in claim 5, said quenching process being a radial cocurrent quenching process.

9. The process as defined in claim 5, said inert gas being preheated prior to introducing said inert gas into said zone between the zones for introducing steam and air.

\* \* \* \* \*

20

25

30

35

40

45

50

55

60

65